

## UNITED STATES PATENT OFFICE

2,665,978

## FUEL OIL COMPOSITIONS

Richard D. Stayner and Robert A. Stayner,  
Berkeley, Calif., assignors to California Research Corporation, San Francisco, Calif., a corporation of Delaware

No Drawing. Application September 25, 1951,  
Serial No. 248,280

7 Claims. (Cl. 44—74)

1

The present invention is concerned with improved hydrocarbon fuels and, more particularly, with hydrocarbon fuels having improved properties as burner fuels and diesel engine fuels.

In the production of burner fuels and diesel engine fuels it is desirable, economically, to employ considerable quantities of cracked refinery stocks. Such stocks are becoming more and more available due to the ever increasing use of thermal and catalytic cracking processes in petroleum refinery operations. When employed in burner fuels and diesel engine fuels these stocks have the disadvantage of forming particles of sludge or gum which tend to deposit and cause plugging of filters, screens and lines. The necessity for frequent interruptions of burner and diesel engine service to replace or unplug clogged filters and screens constitutes a serious problem.

Burner and diesel engine fuel systems ordinarily contain certain amounts of water due to vapor condensation. The presence of this water tends to accelerate the formation of filter plugging gum and sludge in burner and diesel fuels containing cracked stocks and also causes rusting of exposed ferrous metal surfaces, which rust, in turn, eventually loosens and clogs the filters and lines.

Pursuant to the present invention, it has been discovered that by the addition of a small amount of an N,N-di-(alkyl aryl methylene)-N-alkyl-ammonium alkane sulfonate to normally liquid hydrocarbon fuels, any tendency of the fuel to form filter clogging particles of sludge or gum is substantially overcome. Such hydrocarbon fuel compositions, in addition, have the effect of inhibiting rusting of ferrous metal surfaces with which they come in contact, thus substantially eliminating rust particles that may also lead to clogging of fuel oil systems.

The N,N-di-(alkyl aryl methylene)-N-alkyl-ammonium alkane sulfonates employed in the fuel compositions may be illustrated by the following structural formula:



wherein R<sub>1</sub> and R<sub>2</sub> are alkyl groups of from 9 to 18 carbon atoms, Ar is an aryl hydrocarbon group, R<sub>3</sub> is an alkyl group of from 1 to 7 carbon atoms, and R<sub>4</sub> is an alkylene group of from 1 to 7 carbon atoms.

The compounds as illustrated in the above structural formula contain two aryl or alkaryl groups, each of which is connected by a methylene linkage to the nitrogen. Examples of suitable aryl groups are benzene, naphthalene, anthra-

cene, toluene, xylene, mesitylene, etc., with benzene and toluene being preferred for their availability and the high degree of effectiveness characteristic of the compounds containing them. The nuclear alkyl substituents may be straight-chain or branched-chain in nature and may vary from 9 to 18 carbon atoms in length. The alkyl groups may be derived from halogenated hydrocarbons, aliphatic alcohols and olefins including cracked petroleum fractions and polymers of ethylene, propylene and butylene. For present purposes propylene polymers containing from 12 to 15 carbon atoms per molecule are preferred because of their chemical stability derived from the characteristically moderate chain-branching of propylene polymers in general.

The above compounds may be prepared by reacting a molar excess of an alkyl aryl methylene halide with an N-alkyl amino alkane sulfonic acid in the presence of a neutralizing agent. Further and more specific details as to their preparation may be found in copending U. S. application No. 248,279, filed September 25, 1951, of Richard D. Stayner.

In the above structural formula illustrating the invention, that portion derived from the N-alkyl amino alkane sulfonate reactant is represented by the group:

30



Suitable N-alkyl amino alkane sulfonates are sodium N-methyl amino ethane sulfonate, otherwise known as sodium N-methyl taurate, sodium N-ethyl amino ethane sulfonate, potassium N-ethyl 2-amino propane sulfonate, sodium N-butyl amino butane sulfonate, sodium N-hexyl amino cyclohexane sulfonate, etc. Presently preferred is sodium N-methyl amino ethane sulfonate or sodium N-methyl taurate because of its common availability and its particular suitability to the invention.

N,N-dialkylbenzyl-N-methyl taurines constituting the preferred additives of the invention are illustrated by the formula:



wherein  $R_1$  and  $R_2$  are alkyl groups of from 9 to 18 carbon atoms,  $R$  is a hydrogen or methyl group, and  $x$  is an integer of from 1, 2, 3.

This preferred group of additives may be prepared by chloromethylating nuclear alkyl derivatives of benzene, toluene or xylene, for example. A molar excess of the chloromethyl derivative, and preferably at least 2 molar proportions thereof, may then be reacted with sodium  $N$ -methyl taurate at a temperature of from about 50 to 100° C. in the presence of a neutralizing agent such as sodium hydroxide, sodium bicarbonate, sodium carbonate, lime, etc.

Specific examples of  $N,N$ -di-(alkyl aryl methylene)- $N$ -alkyl-ammonium alkane sulfonates within the above generic disclosures which are suitable for incorporation in fuel oil compositions according to the invention are  $N,N$ -di-(nonylbenzyl)- $N$ -methyl-ammonium ethane sulfonate, otherwise known as  $N,N$ -di-(nonylbenzyl)- $N$ -methyltaurine;  $N,N$ -di-(dodecylbenzyl)- $N$ -methyltaurine;  $N,N$ -di-(decyl methyl benzyl)- $N$ -methyltaurine;  $N,N$ -di-(dodecyl methyl benzyl)- $N$ -ethyl ammonium propane sulfonate;  $N,N$ -di-(pentadecyl benzyl)- $N$ -butyl-ammonium butane sulfonate;  $N,N$ -di-(octadecyl di-methyl benzyl)- $N$ -hexyl-ammonium cyclohexane sulfonate;  $N,N$ -di-(nonyl naphthyl methylene)- $N$ -propyl-ammonium hexane sulfonate; and  $N,N$ -di-(dodecyl methyl naphthyl methylene)- $N$ -methyl-ammonium ethane sulfonate, otherwise known as  $N,N$ -di-(dodecyl methyl naphthyl methylene)- $N$ -methyltaurine, etc.

The hydrocarbon fuel base stocks suitable for use in the improved fuel oil compositions of the present invention may be described broadly as petroleum distillates boiling in the range of from about 350° F. to about 750° F. Such distillates are ordinarily characterized by an A. P. I. gravity of at least 20°, and usually at least 25°. The base stocks may be either straight-run distillates or cracked distillates. The present invention finds its greatest utility in hydrocarbon fuels of the preceding types which contain substantial amounts of cracked distillates. Without the additives of this invention such fuels form appreciable amounts of filter plugging sludge and gum which render them unsuitable for use in operations where uninterrupted service is desired, as is the case with most present-day operations.

Very small amounts of the  $N,N$ -di-(alkyl aryl methylene)- $N$ -alkyl-ammonium alkane sulfonates, in the order of 1% by weight or less, have been found to be entirely effective to prevent line and filter clogging and to inhibit rusting when water is present in the system. Amounts in the range of from 0.001 to 0.20 per cent by weight of the total fuel are particularly suitable when the preferred  $N,N$ -di-alkyl benzyl  $n$ -methyltaurines having from 9 to 18 carbon atoms in each of the alkyl groups are employed. Proportions in the range of from 0.005 to 0.015 per cent by weight are most preferred in the more specific embodiments of the invention.

In order to facilitate evaluation of the improved fuel oil compositions of the present invention and avoid an enormous outlay of time and material, a rapid test method for determining filter plugging characteristics was developed. The results of this test method have been found to correlate well with actual field tests using regular fuel oil burners and diesel engines. The test is carried out by mixing 500 ml. of a fuel composition containing 0.01% by weight of additive with 500 ml. of water containing 102 parts per million hardness calcu-

lated as calcium and magnesium carbonates, two-thirds being calcium carbonate. The fuel oil composition and water are shaken in a separatory funnel for 30 seconds, at the end of which they are allowed to stand for 10 minutes. At this point a phase separation occurs and an upper oil layer and a lower water layer are obtained, usually separated by an opaque cuff at their interface. This interface cuff is then filtered through a fritted glass crucible with the aid of a vacuum. Only as much oil and water are filtered as are necessary to assure complete extraction of the cuff, usually about 25 ml. However, in cases of severe emulsions the entire contents of the separatory funnel may have to be filtered. The resultant discoloration of crucible met by the particles of gum and sludge deposited is used as a comparative measure of the hydrocarbon fuel's tendency to plug filters and screens.

In the comparison the filter is compared with a standard series of 11 filters prepared in a similar manner from fuels of known filter plugging tendency. The standard filters are numbered 0 to 10, the higher numbers being identified with the heavier deposits. For convenience, the rating given a particular test sample is termed its interface deposit rating (IFD) and denotes the number of the filter in the standard series with which it compares in amount of filter deposit.

Table I, which follows, shows the IFD values of a number of fuel oil compositions according to the present invention, as compared with a standard diesel or burner fuel. The base fuel employed in each case was a mixture of equal parts of straight run distillate from a waxy base crude boiling in the range of from 384° F. to 675° F. and a Thermofor catalytic cracked fraction boiling in the range of from 376° F. to 566° F.

TABLE I

## Interface filter deposit rating

| Run No. | Additive                                                       | IFD No. |
|---------|----------------------------------------------------------------|---------|
| 1       | $N,N$ -di-( $C_{12}$ -polypropylenebenzyl)- $N$ -methyltaurine | 0       |
| 2       | $N,N$ -di-( $C_8$ -polypropylenebenzyl)- $N$ -methyltaurine    | 2       |
| 3       | $N,N$ -diethylbenzyl- $n$ -methyltaurine                       | 4       |
| 50      | None                                                           | 10      |

The data in Table I clearly shows the marked superiority of the improved hydrocarbon fuel compositions according to the present invention over a conventional diesel or burner fuel. Runs 1, 2 and 3 each show that very little or no filter deposit is obtained from fuel oil compositions containing a representative  $N,N$ -di-(alkyl aryl methylene)- $N$ -alkyl-ammonium alkane sulfonate, whereas the fuel oil base stock itself gives an extremely high filter deposit.

The fuel oil compositions of the present invention were also tested for their rust inhibiting properties. The tests were carried out in accordance with the procedure outlined in ASTM Method D-665-47T. Steel spindles were immersed in an agitated distilled water and fuel oil mixture containing 0.001% by weight of additive and in an agitated sea water and fuel oil mixture containing 0.005% by weight of additive. The base stock fuel was tested in a similar fashion. The results of these tests were as follows:

**5**  
**TABLE II**  
*Anti-rust properties*

| Run No. | Additive                                                        | Anti-rust rating distilled water-oil mixture | Sea water-oil mixture |
|---------|-----------------------------------------------------------------|----------------------------------------------|-----------------------|
| 1.....  | N,N-di-(C <sub>12</sub> -polypropylene-benzyl)-N-methyltaurine. | No rust.....                                 | No rust.              |
| 2.....  | N,N-di-(C <sub>8</sub> -polypropylene-benzyl)-N-methyltaurine.  | Light rust...                                | Do.                   |
| 3.....  | N,N-dikerylbenzyl-N-methyltaurine.                              | .....do.....                                 |                       |
| 4.....  | None.....                                                       | Severe rust...                               | Severe rust.          |

From the above tests it will be readily observed that the improved fuel oil compositions of this invention possess remarkable rust inhibiting properties as compared to ordinary diesel or burner fuels.

The fuel oil compositions according to the present invention may contain other fuel oil additives in addition to the N,N-di-(alkyl aryl methylene)-N-alkyl-ammonium alkane sulfonates. Such additives include: lecithin; oil-soluble alkyl aryl polyglycol ethers, such as didodecyl phenyl dodecaethylene glycol ether; oil-soluble sulfonates, such as the lead salts of petroleum sulfonic acids containing from about 20 to 30 carbon atoms per molecule; oil-soluble naphthenates, such as the alkali metal and lead salts of petroleum naphthenic acids; alkali metal and lead salts of alkyl phenol di-sulfides.

We claim:

1. A hydrocarbon fuel oil composition containing a small amount sufficient to inhibit line and filter clogging and corrosion of an N,N-di-(alkyl aryl methylene)-N-alkyl-ammonium alkane sulfonate in which the alkyl radical of the alkyl aryl methylene groups contains from 9 to 18 carbon atoms, the N-alkyl radical contains from 1 to 7 carbon atoms and the alkane group contains from 1 to 7 carbon atoms.

2. A hydrocarbon fuel oil composition contain-

**6**

ing a small amount sufficient to inhibit line and filter clogging and corrosion of an N,N-di-alkyl benzyl N-methyl taurine having from 9 to 18 carbon atoms in each of the alkyl groups.

3. A hydrocarbon fuel oil composition containing a small amount not exceeding 1% by weight of an N,N-di-alkyl benzyl N-methyl taurine having from 9 to 18 carbon atoms in each of the alkyl groups.

10 4. A hydrocarbon fuel oil composition comprising a major proportion of a normally liquid hydrocarbon fuel oil boiling in the range of from about 350° F. to about 750° F. and a small amount not exceeding 1% by weight of an N,N-di-alkyl benzyl N-methyl taurine having from 9 to 18 carbon atoms in each of the alkyl groups.

15 5. A hydrocarbon fuel oil composition comprising a major proportion of a normally liquid hydrocarbon fuel oil boiling in the range of from about 350° F. to about 750° F. and from 0.005 to 0.015 per cent by weight of an N,N-di-alkyl benzyl N-methyl taurine having from 9 to 18 carbon atoms in each of the alkyl groups.

20 6. A hydrocarbon fuel oil composition comprising a major proportion of a normally liquid hydrocarbon fuel oil boiling in the range of from about 350° F. to about 750° F. and from 0.005 to 0.015 per cent by weight of an N,N-di-alkyl benzyl N-methyl taurine having a propylene polymer of 12 to 15 carbon atoms as each of its alkyl groups.

25 7. A hydrocarbon fuel oil composition as described in claim 6, wherein the normally liquid hydrocarbon fuel oil contains a substantial proportion of cracked petroleum distillate.

RICHARD D. STAYNER.  
ROBERT A. STAYNER.

References Cited in the file of this patent

UNITED STATES PATENTS

Number Name Date  
2,433,997 Linch Jan. 6, 1948